

June 4, 1935.

J. G. BOWDEN

2,003,917

HANDLE GRIP

Filed Jan. 24, 1933



INVENTOR:

*James G. Bowden,*  
BY  
*J. H. McCrea,*  
his ATTORNEY.

## UNITED STATES PATENT OFFICE

2,003,917

## HANDLE GRIP

James G. Bowden, Millbury, Mass., assignor to  
 The Felters Company, Boston, Mass., a corporation of Massachusetts

Application January 24, 1933, Serial No. 653,286

3 Claims. (Cl. 273—75)

This invention relates to grips for the handles of tennis rackets, golf clubs, and various other implements and tools, and also to the materials used in making such grips.

Control of a tennis racket, golf club, or the like, is greatly facilitated if the handle has the desired "feel". Usually this means a certain but very limited degree of tackiness sometimes combined with a slight "give" or yielding quality. Naturally the requirements for a grip vary considerably with the nature of the implement on which it is used, and to some extent, also, with the desires of different players. For example, a large proportion of the tennis players prefer to have only a slight degree of tackiness in the racket handle grip, and they want a handle which is very firm, with practically no give or yielding characteristics. Any great degree of tackiness interferes with the proper execution of the strokes and slows up the shifting of the racket in the hand which many players make in changing from a fore-hand to a back-hand stroke, or vice versa. Essentially the same qualities are desirable in a squash racket handle, but a greater degree of yield or give is permissible there and is preferred by a large proportion of the players. In a golf handle grip more yield is permissible in most cases and a higher degree of tackiness is preferred by many players than would be permissible in a tennis racket grip.

Various kinds of rubber, fabric and leather grips have been proposed to meet these requirements but few of them have gone into use to any substantial extent. As a rule leather which has been impregnated with oils and other constituents to give up the desired feel is used most commonly for the handles of golf clubs and squash rackets, while tennis racket handles are generally used bare, no grip having been devised for them which meets the requirements of any substantial percentage of the players. While the leather grip thus is very satisfactory for some purposes, it is open to the objection that in a relatively short time it either loses the constituents which give the desired tacky feel, or else these constituents undergo some change which undesirably modifies the feel of the grip.

The present invention aims to devise a grip which will meet a wider range of needs than those heretofore available, and which will have a high degree of stability and uniformity.

I have found that an exceptionally satisfactory material for grips can be made by impregnating felt with a suitable rubbery compound serving to bind the fibers of the felt securely together but

without destroying completely the fibrous or felty feel of the original goods. A particularly satisfactory article can be made by impregnating a sheet of felt with vulcanized rubber latex, drying the goods so impregnated, and then cutting them into strips or other sections suitable for application to a handle. Preferably an all wool felt is used, although other fibers can, if desired, be associated with the wool fibers in very substantial proportions. The best results are produced by using a true felt in which the fibers are interlocked by a characteristic felting action. This necessarily means a wool felt but not necessarily an all wool goods. For most purposes a felt having a thickness of in the neighborhood of one-sixteenth of an inch is satisfactory, although the latex will readily penetrate greater thicknesses and the thickness may be determined entirely in accordance with the requirements of individual uses. No modification of the felt making operation is required for this purpose. The vulcanized latex used may be that readily obtainable on the market as vulcanized latex or that sold under the name of "Vultex". Usually these materials contain in the neighborhood of 35% or 40% of rubber dispersed in a natural serum consisting chiefly of water, but containing, also, some other ingredients. Small proportions of protective colloids may be added to the dispersion in order to prevent coagulation and to give added stability, the latex usually containing also a small proportion of ammonia which acts as a preservative.

When a sheet of felt impregnated in the manner above described has been dried sufficiently to drive off the water and other volatile constituents of the latex, it will be found that the fibers are permanently bonded to each other by the vulcanized latex rubber left in the goods. At the same time the fibers in the fabric are still prominent and the felty feel of the fabric is still retained to a substantial degree. The extent to which these properties are affected will depend in a large measure on the proportion of rubber added to the goods, and it is desirable to use a sufficient proportion of rubber to produce the desired bonding of the fibers and to give the necessary tackiness while still retaining the felty appearance and much of the felty structure of the goods. I have found that in treating a web of all wool felt seventy-two inches wide and approximately one-twentieth of an inch thick, very good results are obtained by allowing the felt to take up approximately four-fifths of a gallon of vulcanized latex to the running yard, the latex containing from 35% to 40% of solids. The pro-

portion of rubber so added to the goods may, however, be varied within very substantial limits while still producing very satisfactory results.

Various constituents may be added to the latex 5 in order to produce special results. For example, pigments may be added to control the color within reasonable limits. Fillers may be added to control the degree of tackiness, and the proportion of the dispersing medium naturally will be 10 varied in accordance with the concentration required. In fact, variation of the concentration is a convenient means for controlling the quantity of rubber added to the goods. For some purposes it will be found desirable also to add adhe- 15 sives such as casein, glue, or the like, to the latex in order to improve the bond between the latex and fibers as well as to modify the characteristics of the finished product.

The impregnating operation may be carried out 20 in various ways. A convenient method consists in running the goods through an impregnating bath at such a speed that it can take up the desired quantity of latex, passing the sheet between squeeze rolls to remove the excess material, and 25 then drying the impregnated sheet at a moderate heat, say for example, 150° to 175° F. Usually the surface of the goods is rough and harsh after being dried, and it can be substantially improved by pressing the dried sheet between plates heated 30 to in the neighborhood of 120° F. Often it is more convenient to cut the goods into sheets approximately a yard square before pressing them. A pressure of a ton to the square foot is ample for present purposes, the pressure being 35 maintained for perhaps a minute or a minute and a half. In some cases a difficulty occurs in this operation, due apparently to the presence of moisture, and when this happens it can be readily overcome by shortening the pressure period to, 40 say, one-half or three-quarters of a minute, but repeating it once or twice until the desired results are obtained. The pressing operation removes the surface irregularities, reduces the entire body to an approximately uniform thickness, and produces a more agreeable surface. 45 Later the sheets can be slit or cut into strips of suitable width, and at some stage in the process the goods may conveniently be run across a knife edge to partly free the ends of the surface fibers 50 from the main body of the goods and to break up or largely destroy the glaze-like surface characteristic which the treated felt frequently has after coming out of the pressing operation.

Some difficulty usually is experienced in securing a uniform impregnation of a high grade all wool felt with rubber latex due apparently to the tendency of the goods to strain out the rubber particles. I have found, however, that this difficulty can be effectively overcome by giving the goods a preliminary treatment with some agent which serves to promote penetration and which may, therefore, be termed a penetrating agent. While the action of these penetrating agents on the goods is not thoroughly understood, they apparently have the effect of so reducing the surface tension of the latex that it penetrates readily into the felt. Such penetrating agents may consist of sulphonated alcohols or the aromatic or hydroaromatic sulphonic acids or salts, examples of which are formaldehyde, naphthalene or alkyl naphthalene sulphonic acid. The sulphuric ester of butyl ricinoleic acid is suitable for this purpose.

The penetrating agent which I have used with

the best results is known as NeKal BX dry sold by the General Dyestuff Corporation. My method of procedure has been to run the goods through a bath of this agent, and then, while they are still wet, to run them through the latex bath. The goods could, however, be dried, if desired, between the two baths but this ordinarily is not desirable.

While I have obtained the best results by the use of vulcanized rubber latex, it will be evident that rubber can be added to the felt in other ways. For example, the felt can be impregnated with ordinary or unvulcanized latex and the rubber subsequently vulcanized at temperatures well below those liable to damage the fiber of the felt. The so-called "cold" vulcanizing processes 10 may be used for this purpose and are well known to the rubber art. The impregnation may also be produced by dissolving the rubber in a suitable solvent and immersing the felt in the solution. Impregnation is effected more readily, however, 15 with latex than with a rubber solution, and the use of volatile solvents also is avoided.

Typical embodiments of the invention are illustrated in the accompanying drawing in which,

Figure 1 is a plan view of a tennis racket having 25 a handle provided with a grip portion embodying features of this invention;

Fig. 2 is a perspective view of a strip of felt made in accordance with this invention; and

Fig. 3 is a perspective view of a small section of 30 the strip shown in Fig. 2 but greatly enlarged.

Figs. 2 and 3 show a strip 2 of unwoven felt in which the fibers are interlocked with each other by the felting operation, and Fig. 3 attempts to show the rubber bonding the fibers together and 35 producing a firmer and more substantial sheet which still retains, however, certain of its felty characteristics. Such a strip wound around the handle of a racket is illustrated in Fig. 1 at 3.

The grip provided by this invention is substantially homogeneous in construction, is unaffected by any ordinary conditions of use, wears down very uniformly and without changing substantially in characteristics, and is therefore extremely stable.

Having thus described my invention, what I desire to claim as new is:

1. A handle grip comprising a flexible strip of wool felt, the fibers of which are elastically bonded permanently together with a rubbery material, 50 the proportion of said material being so limited that a substantial portion of the felty feel and fibrous characteristics of the felt are retained.

2. A handle grip comprising a flexible strip of wool felt impregnated with a sufficient proportion of latex rubber to bond the fibers of the felt together, the quantity of the rubber being so limited as to preserve a substantial portion of the felty feel of the goods.

3. A handle grip comprising a flexible strip of 60 wool felt of approximately uniform thickness impregnated substantially throughout the entire body thereof with vulcanized latex rubber, the proportion of the rubber being so limited as to bond the fibers together at their intersections 65 while still preserving the fibrous nature of the goods, and the surface of the impregnated material being characterized by the presence of fibers partially freed from adjacent fibers and binder and giving the impregnated material a 70 felty feel.

JAMES G. BOWDEN.